

G. GRÖNDAL.

**METHOD OF CONCENTRATING ORE BY FLOTATION.**  
**APPLICATION FILED JAN. 18, 1916.**

1,202,512.

Patented Oct. 24, 1916.



**INVENTOR**

By Gustaf Grindal  
Kamm and Kamm  
ATTORNEYS

# UNITED STATES PATENT OFFICE.

GUSTAF GRÖNDAL, OF DJURSHOLM, SWEDEN, ASSIGNOR TO BEER, SONDEIMER & CO.,  
OF FRANKFORT-ON-THE-MAIN, GERMANY.

## METHOD OF CONCENTRATING ORE BY FLOTATION.

1,202,512.

Specification of Letters Patent.

Patented Oct. 24, 1916.

Application filed January 18, 1916. Serial No. 72,757.

*To all whom it may concern:*

Be it known that I, GUSTAF GRÖNDAL, a subject of the King of Sweden, and resident of Djursholm, Sweden, have invented a certain new and useful Improved Method of Concentrating Ore by Flotation, of which the following is a specification.

In using the known oil flotation method for concentrating very finely subdivided ore materials it has been found that the oil does not well moisten all the particles. Hitherto the oil has been brought into intimatest possible contact with the particles of mineral by means of stirring. The grains of mineral not moistened by the oil generally are lost. By long experiments I have succeeded in removing the difficulty of moistening the subdivided material with oil.

My invention consists in distributing the oil in a streaming elastic fluid under pressure such as steam or air and afterward mixing the steam or air under pressure with its contents of oil with a large quantity of an elastic fluid such as air or any other gas and then pressing the mixture into water holding the ore powder suspended. In this manner an emulsion is produced, whereby, when the air is driven through this emulsion, there is created a large number of air bubbles each surrounded by a thin film of oil, which bubbles when pressed through the suspended ore come with their oily films in contact with the respective particles of ore which then become moistened with oil. By the extremely energetic stirring caused by blowing the bubbles through the suspended ore a new technical result is obtained as in order to attain the object aimed at one need only use a very small proportion of oil.

A form of apparatus suitable for carrying the method into effect is shown on the accompanying drawing as an example only.

The figure shows a vertical section through the apparatus.

By means of a pipe *a* the necessary quantity of oil is fed into a Körting steam jet apparatus *b* beneath or near the mouth of a steam conduit *c* from a source of steam not shown. The steam under pressure during its passage through *b* draws in a large quantity of air. The mixture of air and steam mixed with oil is then pressed through the pipe *e* provided with a funnel shaped outlet

*d* into the reservoir *f*, said reservoir by means of the pipe *g* opening above the funnel *d* being continually fed with ore powder suspended in water.

In the reservoir *f* an energetic intermixture is effected by which the oil comes into intimate contact with the mineral of ore. Air in abundant quantity being present the oily particles of ore float up to the surface. Over the partition *h* the mixture of ore thus treated flows to the Callow cone *i* from which the ore concentrate flows off over the overflow *k* into the channel *l* and the refuse through a valve *m*. If required the refuse is led into a similar apparatus and is treated once more in the manner described above.

In the following claims I use the phrase "gaseous medium" in a sense broad enough to include steam, air or other elastic fluid subject to compression.

I claim:

1. The flotation method consisting in projecting a heated gaseous current having a selective agent diffused therein against an opposed current or ore pulp, and collecting by flotation the particles thereby differentiated.

2. The method herein described of concentrating finely divided ore by means of oil flotation, said method consisting, essentially, in first distributing oil in a stream of heated gas under pressure and thereby atomizing the oil, then utilizing the flow of the gas-oil to commingle therewith a large quantity of another gas, and forcing the gas-oil mixture thus formed into a liquid against a countercurrent of finely divided ore.

3. The flotation process herein described which consists, essentially, in atomizing an oleaginous agent by the action of a gaseous medium under pressure and producing thereby a gaseous suspension; utilizing the flow of the gaseous suspension to induce the commingling therewith of a large body of another gas; and injecting the combined gaseous fluid into a hydraulic body against a counterflow of pulverized ore particles.

4. The flotation process herein described which consists, essentially, in atomizing an oleaginous agent by the action of a heated gaseous medium to atomize said agent and produce therefrom a gaseous suspension; utilizing the flow of said gaseous suspension

to induce the commingling therewith of a  
large volume of another gaseous medium;  
and projecting the combined fluid up-  
wardly through a hydraulic body and  
against a counterflow of pulverized ore par-  
ticles.

In testimony whereof I have signed my

name to this specification, in the presence of  
two subscribing witnesses.

GUSTAF GRÖNDAL.

Witnesses:

FRANK LYON,  
GRETA PRIEN.